

## CREASE-PROOFING CELLULOSIC FABRICS, THE FABRICS OBTAINED AND METHODS OF MAKING THEM

Colin L. Browne, Charlotte, N.C., assignor to Rohm & Haas Company, Philadelphia, Pa., a corporation of Delaware

No Drawing. Filed Jan. 29, 1957, Ser. No. 636,852

19 Claims. (Cl. 8—116.2)

The present invention relates to an improved process for the treatment of cellulosic fabrics, especially cotton and rayon, for the purpose of increasing resistance to creasing, to crushing, wrinkling, and of reducing the tendency to shrinkage on laundering. The invention is particularly concerned with the process of crease-proofing cellulosic fabrics or other textile materials of cellulosic type and to the improved products obtained.

It is an object of the present invention to provide a process for increasing the resistance of cellulosic fabrics to creasing, crushing, and wrinkling by means of a cross-linking agent, which, in reacting with the cellulosic materials, does not form a resin on the textile materials so that it effects the crease-proofing and so on without essentially modifying the hand or optical characteristics of the textile material. Another object of the present invention is to provide a process for increasing the resistance to creasing and the like of cellulosic textiles by means of cross-linking agents which enhance the receptivity of the textile materials to dyeing. While such an improvement in receptivity to acid dyes might be expected because of the basic nature of the cross-linking agent, the surprising discovery has been made that the cross-linked products of the present invention also have markedly improved receptivity to other conventionally used classes of dyestuffs, such as direct dyes and especially to acid dyes. Another object of the invention is to provide improved modified cellulosic textiles. Other objects and advantages of the invention will be apparent from the description thereof hereinafter.

The use of thermosetting resin-forming condensates, such as those of formaldehyde with urea, melamine or other nitrogen-containing compounds, for the purpose of increasing the resistance of cellulosic fabrics to creasing and the like is known. These resin-forming materials, however, are generally characterized by the deposition of a substantial amount of resin on the surface of the fibers of the textile material which modifies the hand, frequently in a disadvantageous manner, as by harshening the hand or feel of the textile material.

In accordance with the present invention, cellulosic fabrics are improved in their resistance to creasing, crushing, wrinkling, and tendency to shrink on washing by reaction with the salt of a poly(vinyloxyalkyl) amine which, under the conditions of reaction, reacts exclusively with the hydroxyl groups of the cellulosic molecules in the textile material and does not form a resin deposit on the surface of such fibers or in or on the textile fabric. The poly(vinyloxyalkyl) amine, the salt of which is used for effecting the reaction of the present invention may be any of those having the general Formula I:



where

$n$  is an integer having a value of 2 to 3,

$R$  is selected from the group consisting of cyclohexyl, benzyl, and alkyl groups having 1 to 8 carbon atoms,

A is an alkylene group having 2 to 4 carbon atoms, and

X is selected from the group consisting of O and S.

In the formula, at least two carbon atoms of the alkylene group extend in a chain between the X atom and the nitrogen atom. Examples of alkylene groups that may be employed include ethylene, trimethylene, propylene, in which one of the carbon atoms of the ethylene group extending between the X and N atoms is substituted by a methyl group, and isobutylene, where one of the carbon atoms of the ethylene group extending between the nitrogen and X atoms is substituted by two methyl groups. The alkyl groups which may represent R include methyl, ethyl, n-propyl, isopropyl, n-butyl, isobutyl, sec-butyl, t-butyl, hexyl, n-octyl, and t-octyl.

The salts of the amine may be formed from any suitable acid such as inorganic or mineral acids, of which hydrochloric acid, phosphoric acid, nitric acid, sulfuric acid, and perchloric acid are representative, or it may

20 be any organic acid, such as a monobasic acid of the aliphatic series, including formic acid, acetic acid, propionic acid, and so on, or it may be a polycarboxylic acid, such as maleic acid, fumaric acid, succinic acid, citric acid, adipic acid, sebacic acid, oxalic acid, phthalic acid, or tartaric acid. If desired, the salt may be formed by the use of a mixture of two or more different acids, such as a mixture of an organic acid with a mixture of an inorganic or mineral acid in any desired proportions.

30 The amines of Formula I are generally insoluble in water but the salts conveniently are quite water-soluble. The salts may be prepared by simply dispersing the amine in water with agitation and adding acid during the agitation until the amine is completely dissolved. Of the

35 various acids mentioned hereinabove, the preferred salts are obtained by the use of formic acid, acetic acid, maleic acid, nitric acid, fluoboric acid, or perchloric acid as the treated fabrics obtained using the amine salts of these acids exhibit negligible or a complete absence of

40 discoloration as a result of the treatment. The amine salts of the other acids are useful, however, when dyed or otherwise colored textile materials are treated where the discoloration is not noticeable.

The amine salt may be applied to the textile material in any suitable way. Thus, an aqueous solution thereof

45 having any desired concentration may be prepared and the textile material may be treated with such solution by dipping, spraying, brushing, by transfer rollers, by the use of a textile pad or any other suitable and conventional equipment or system. Generally, after the solution is applied, excess may be removed as by squeezing or squeegeeing. When application is by a procedure where approximately 100% wet pick-up occurs, the concentration of the salt may be from 5 to 20% for most purposes. Optimum results are generally obtained when

50 8 to 12% concentration of the salt in the aqueous system is applied at about 100% wet pick up. After application and any desired removal of excess, the textile material is dried. This may be effected simply by drying in ambient air or by the application of heated air, by infrared heat, or by high frequency electric induction procedures. The particular equipment employed may be selected depending upon the particular type of textile material treated.

55 The treatment of the present invention may be applied to any textile material containing cellulosic fibers or

yarns and the textile material may be in the form of woven or knitted fabrics, "non-woven" fabrics derived from carded webs or from fibrous or filamentous webs obtained in any suitable fashion, such as air-deposition, wherein the fibers or filaments are distributed in a haphazard array. The treatment may also be applied to

yarns, threads or other plied structures, or it may be applied to fibers or filaments in the form of loose or bulk masses or in the form of more or less compacted webbing, matting, or batting. In all fibrous structures having the fibers in heterogeneous array, the treatment renders the textile more resilient.

The fabrics or fibrous masses that may be treated are those which contain a predominant proportion of cellulosic fibers and/or filaments, by which is meant that the cellulosic fibers constitute more than 50% of the total fibers by weight. It is particularly useful with textile materials of cotton, viscose rayon, cuprammonium cellulose rayon, linen, ramie, as well as textile materials comprising fibers and filaments of two or more of such cellulosic materials. At the time of treatment with the cross-linking agent of the present invention, the fabric may be in the greige state or it may have been previously bleached, dyed, and/or printed with pigments or otherwise finished.

After the drying of the fabric to which the amine salt has been applied, it must be subjected to a heating step in which the amine reacts with the cellulose by addition of the unsaturated group to the hydroxyl group of the cellulose to form an acetal linkage between the cross-linking bridge and the cellulose molecules. The heating should be in a range of temperature from about 250° to 400° F. for a period of about one-half minute to an hour, the shorter time being used with the higher temperature and vice versa. In any case, the upper limit of temperature should not be so high as to damage the fibers in the fabric by thermal decomposition. Preferably, a temperature of 300° to 350° F. is employed. At a temperature of 325° F., a short period of about 2½ to 3 minutes is entirely adequate, whereas at 300° F. the time generally needed is about 15 minutes. The amine salt is self-catalytic in that no other material is needed to effect the reaction between the cellulose and the cross-linking agent at the elevated temperature specified.

As mentioned hereinbefore, the cross-linking agents of the present invention do not appreciably modify the hand or feel of the textile material. They also improve receptivity to acid dyes. The cross-linked textiles are quite resistant to alkaline materials and, on being subjected to heat, they undergo substantially no loss in strength even when such heat is elevated to a scorching temperature where discoloration is effected.

If desired, the treatment with the amine salt may be supplemented by a treatment with a hand-modifier or builder, softened, water-repellent agents, or materials which enhance the crease-resistance that can be obtained by means of the cross-linking agent. Such modifying agents may be applied simultaneously by way of the same aqueous solution of the salt or they may be applied to the fabric before or after the application of the amine salt by means of a separate operation. Such additional modifying agents may be applied advantageously by a separate operation after the completion of the cross-linking by means of the amine of the present invention.

As water-repellent materials which also serve to soften the textile material, there may be used those quaternary ammonium compounds having a long-chain hydrocarbon group, such as stearyl pyridinium chloride, octadecyl oxy-methylpyridinium chloride, and the various quaternary ammonium salts described in U.S. Patent 2,351,581. These quaternary ammonium salts are water-soluble in the salt form and they can, therefore, readily be included within the aqueous solution of the amine salt. The amount of water-repellent or softener may be as much as 5% and is preferably in the range of about 1 to 3% in the aqueous medium by which it is applied, assuming 100% wet pick up. When it is applied solely for the purpose of softening, there may be employed as little as 0.1%.

Examples of auxiliary agents for enhancing the crease-

resistance which can be applied in aqueous media include aqueous dispersions of water-insoluble linear addition polymers of one or more monoethylenically unsaturated monomeric compounds. Examples include water-insoluble copolymers of 0.5 to 8% by weight of acrylic acid, methacrylic acid, and itaconic acid. Any one or more of these monoethylenically unsaturated acids may be copolymerized with one or more other copolymerizable compounds containing a single vinylidene group, such as esters of acrylic acid or methacrylic acid and monohydric alcohols such as methyl, ethyl, butyl, octyl, dodecyl, cyclohexyl, cyanoethyl, aminoethyl, and the like; esters of itaconic acid and the above alcohols; esters from maleic, fumaric or citraconic acids, and the above alcohols; vinyl esters of carboxylic acids such as acetic, propionic, butyric, and the like; vinyloxyalkyl esters such as vinyloxyethyl acetate, etc.; vinyl ethers such as ethyl vinyl ether, butyl vinyl ether, octyl vinyl ether, hydroxyethyl vinyl ether, aminoethyl vinyl ether, aminopropyl vinyl ether, dimethylaminoethyl vinyl ether, vinyloxyethoxyethanol, vinyloxypropoxyethanol; methacrylonitrile or acrylonitrile, acrylamide, or methacrylamide, and N-substituted amides of these types; vinyl chloride, vinyl bromide, vinylidene chloride, vinylidene fluoride, vinylidene cyanide, 1-chloro-1-fluoroethylene, ethylene, styrene, 2-vinylpyridine, 4-vinylpyridine, 2-methyl-5-vinylpyridine. These water-insoluble copolymers may be dispersed by means of non-ionic dispersing agents, such as alkylphenoxypropoxyethoxyethanols having alkyl groups of about seven to eighteen carbon atoms and six to sixty or more oxyethylene units, such as heptylphenoxypropoxyethoxyethanols, octylphenoxypropoxyethoxyethanols, methyl-octylphenoxypropoxyethoxyethanols, nonylphenoxypropoxyethoxyethanols, dodecylphenoxypropoxyethoxyethanols, and the like; polyethoxyethanol derivatives of methylene linked alkyl phenols; sulfur-containing agents such as those made by condensing six to sixty or more moles of ethylene oxide with nonyl, dodecyl, tetradecyl, t-dodecyl, and the like mercaptans or with alkylthiophenols having alkyl groups of six to fifteen carbon atoms; ethylene oxide derivatives of long-chained carboxylic acids, such as lauric, myristic, palmitic, oleic, and the like or mixtures of acids such as found in tall oil containing six to sixty oxyethylene units per molecule; analogous ethylene oxide condensates of long-chained alcohols, such as octyl, decyl, lauryl, or cetyl alcohols; ethylene oxide derivatives of etherified or esterified polyhydroxy compounds having a hydrophobic hydrocarbon chain, such as sorbitan monostearate containing six to sixty oxyethylene units, etc.; block copolymers of ethylene oxide and propylene oxide comprising a hydrophobic propylene oxide section combined with one or more hydrophilic ethylene oxide sections. The concentration of the water-insoluble polymers may be from ½ to 5% in the aqueous medium by which it is applied, either simultaneously with the amine salt or before or after the application of the amine salt. These auxiliary crease-proofing agents may be used in amounts which serve to modify the hand from a soft to a firm or stiff hand depending upon what is desired and depending upon the selection of comonomers used in any copolymer thus applied.

The fabric treated in accordance with the present invention may be a dyed fabric but, if not, the pigments and/or dyes may be included in the aqueous solution used to apply the cross-linking agent or any other auxiliary treating agent. A dye or pigment may be applied by printing or dyeing the fabric after the completion of the crease-proofing treatment of the present invention.

In the following examples, which are illustrative of the present invention, the parts and percentages are by weight unless otherwise indicated. The tests whose results are given in the examples are performed on the treated fabric after being conditioned at 70° F. and 65% relative humidity. The crease-recovery angle is the angle obtained by the standard method of testing therefor. The tensile strength

is the raveled strip tensile strength obtained on an Instron tester and is given in units of lbs./inch, and the Elmendorf tear strength is given in scale units which can be converted to pounds by multiplying by 0.035. In all cases, unless otherwise indicated, the values given for the test are the average for the values of the warp and filling.

EXAMPLE 1

(a) 7.5 ml. of methyl(di-(2-vinyloxyethyl))amine are suspended with stirring in 50 ml. of water yielding a pH of about 10 to 11. Then a solution in water of formic acid having a concentration of 50% is added until the amine dissolves (about 5 to 6 ml. being required), yielding a pH of 5 to 6. The solution is then diluted to 100 ml. and at this concentration is applied at 100% wet pick-up to an 80 by 80 cotton fabric. The treated fabric after removal of excess solution is dried by heating for five minutes at 240° F. and is cured for five minutes at 325° F. It is then washed with an alkaline detergent, dried, conditioned, and tested. Table A compares the properties tested of treated and untreated fabrics.

Table A

|                                        | Untreated Fabric | Treated Fabric |
|----------------------------------------|------------------|----------------|
| Crease-Recovery Angle.....degrees..... | 69               | 112            |
| Tensile Strength.....                  | 43.0             | 29.1           |
| Elmendorf Tear Strength.....           | 35               | 22             |

The treated fabric is dyed with Orange II (Color Index No. 151) and takes on a deep orange color much deeper than the untreated fabric dyed under the same conditions with the same dye.

(b) In the same way, a fabric having a similarly improved crease-recovery angle is obtained by the procedure of part (a) substituting 7.5 ml. of methyl(di-(2-vinylthioethyl))amine.

(c) The procedure of part (a) is repeated substituting 7.5 ml. of n-butyl(di-(2-vinyloxyethyl))amine for the amine used in part (a). Results: Crease-recovery angle 110°, tensile strength 26.5, and Elmendorf tear strength 2. The treated fabric is dyed with Direct Brilliant Blue SBC (Color Index No. 466). A deep blue shade is obtained whereas the untreated fabric is tinted only to a very light blue shade.

(d) The procedure of part (a) is repeated with similar results substituting 7.5 ml. of cyclohexyl(di-(2-vinyloxyethyl))amine for the amine of part (a).

(e) In the same way, a fabric having a similarly improved crease-recovery angle is obtained by the procedure of part (a) substituting 7.5 ml. of benzyl(di-(2-vinylthioethyl))amine.

(f) In the same way, a fabric having a similarly improved crease-recovery angle is obtained by the procedure of part (a) substituting 7.5 ml. of n-octyl(di-(2-vinylthioethyl))amine.

EXAMPLE 2

The procedure of Example 1 is repeated except that the amine is replaced with 10 ml. of tri(2-vinyloxyethyl)amine. The pH after neutralization with the formic acid in this case is between 3.5 and 4.5.

Table B

|                                        | Untreated Fabric | Treated Fabric |
|----------------------------------------|------------------|----------------|
| Crease-Recovery Angle.....degrees..... | 71               | 121            |
| Tensile Strength.....                  | 42.3             | 25.6           |
| Elmendorf Tear Strength.....           | 35               | 19             |

EXAMPLE 3

(a) 15 ml. of methyl(di-(2-vinyloxyethyl))amine are suspended in 50 ml. of water and neutralized with 25%

aqueous formic acid yielding a pH of 5.5 to 6. After dilution to 100 ml., an 80 by 80 cotton fabric is treated with the solution as in Example 1, except the drying is effected in air instead of at 240° F. The results of the tests are as follows:

Table C

|                                        | Untreated Fabric | Treated Fabric |
|----------------------------------------|------------------|----------------|
| Crease-Recovery Angle.....degrees..... | 69               | 116            |
| Tensile Strength.....                  | 39.7             | 26.5           |
| Elmendorf Tear Strength.....           | 43               | 19             |

(b) The procedure of part (a) hereof is repeated except that three ml. of an aqueous dispersion of poly(butyl acrylate) (35% solids) is added to the neutralized solution before dilution to 100 ml. The treated fabric has a crease-recovery angle of 130°, a tensile strength of 21.3 lbs./inch and a tear strength of 27.

(c) The procedure of part (a) hereof is repeated except that before conditioning the treated fabric for testing it is padded through an aqueous dispersion containing 1% of poly(butyl acrylate) obtained by dilution of an emulsion polymer thereof. The application of this dispersion is effected at 100% wet pick-up, the fabric is dried five minutes at 240° F., cooled and then conditioned. It has a crease-recovery angle of 131°, a tensile strength of 21.3 lbs./inch and a tear strength of 27.

EXAMPLE 4

5 ml. of methyl(di-(2-vinyloxyethyl))amine are suspended in 50 ml. of water and neutralized with 30% aqueous acetic acid to a pH of about 6 and diluted to about 100 ml. The resulting solution is applied to an 80 by 80 cotton fabric at 100% wet pick up, and after treatment was brought to 325° F. for ten minutes to effect drying and cross-linking. After washing, drying and conditioning, the results are tabulated:

Table D

|                                        | Untreated Fabric | Treated Fabric |
|----------------------------------------|------------------|----------------|
| Crease-Recovery Angle.....degrees..... | 75               | 112            |
| Tensile Strength.....                  | 38.9             | 28.4           |
| Elmendorf Tear Strength.....           | 34               | 24             |

EXAMPLE 5

The procedure of Example 4 is repeated except that 20 ml. of methyl(di-(2-vinyloxyethyl))amine are used instead of 5 ml. The treated fabric obtained has a crease-recovery angle of 99°, a tensile strength of 30.6 lbs./inch and a tear strength of 26.

EXAMPLE 6

10 ml. of methyl(di-(2-vinyloxyethyl))amine are suspended with stirring in 40 ml. of water. Several solutions are made in this way and then neutralized to a pH of 6 with a 5 N solution of each of the following acids. After dilution to 100 ml., a separate 80 by 80 cotton fabric is treated in each of the solutions and the procedure of Example 4 is followed. In the following table, the results of testing the conditioned fabric are presented alongside the respective acid used and the treatment.

Table E

| Acid          | Crease-Recovery, degrees | Tensile Strength | Elmendorf Tear Strength |
|---------------|--------------------------|------------------|-------------------------|
| Acetic.....   | 108                      | 28.4             | 23                      |
| Citric.....   | 115                      | 28.9             | 23                      |
| Formic.....   | 115                      | 26.7             | 22                      |
| Maleic.....   | 112                      | 27.8             | 23                      |
| Tartaric..... | 115                      | 26.3             | 21                      |

7  
EXAMPLE 7

The procedure of Example 6 is followed using each of several solid acids instead of 5 N solutions. The results obtained are presented in Table F.

Table F

| Acid     | Crease-Recovery, degrees | Tensile Strength | Elmendorf Tear Strength |
|----------|--------------------------|------------------|-------------------------|
| Oxalic   | 119                      | 25.9             | 22                      |
| Phthalic | 103                      | 30.1             | 25                      |
| Succinic | 108                      | 27.9             | 23                      |

## EXAMPLE 8

10 ml. of methyl(di-(2-vinyloxyethyl))amine are suspended in 40 ml. of water and neutralized to a pH of 6 with 5 N solutions of the following inorganic acids. After dilution to 100 ml. and application at 100% wet pick-up to an 80 by 80 cotton fabric, each fabric thus treated is heated at 325° F. for 10 minutes to effect drying and cross-linking. After washing, drying and conditioning, the results obtained are as indicated in the following table:

Table G

| Acid         | Crease-Recovery, degrees | Tensile Strength | Elmendorf Tear Strength |
|--------------|--------------------------|------------------|-------------------------|
| Sulfuric     | 127                      | 25.7             | 19                      |
| Hydrochloric | 119                      | 22.3             | 18                      |
| Phosphoric   | 120                      | 23.5             | 20                      |
| Nitric       | 98                       | 24.0             | 20                      |
| Fluoboric    | 98                       | 28.7             | 23                      |
| Perchloric   | 108                      | 25.0             | 21                      |

## EXAMPLE 9

Sixty parts of a 25% solution of formic acid in water is mixed with 40 parts of a 25% solution of sulfuric acid in water and used to neutralize a suspension of 10 ml. of methyl(di-(2-vinyloxyethyl))amine in 50 ml. of water to a pH of 6. After dilution to 100 ml., an 80 by 80 cotton fabric is treated with the solution at 100% wet pick-up, air-dried, and then heated five minutes at 325° F. It is washed, dried and conditioned. The crease-recovery angle of the warp is 126°, the tensile strength of the warp is 29.2 lbs./inch and the Elmendorf tear strength across the warp is 30.

## EXAMPLE 10

20 ml. of methyl(di-(2-vinyloxyethyl))amine are suspended in 40 ml. of water and neutralized to a pH of 5.5 using 25% aqueous formic acid. The solution is diluted to 100 ml. and a rayon fabric is treated at 100% wet pick-up with the solution, air-dried, heated five minutes at 325° F., washed, dried and conditioned. The results are presented in the following table. Reference to tests on the warp only.

Table H

|                                   | Untreated Fabric | Treated Fabric |
|-----------------------------------|------------------|----------------|
| Crease-Recovery Angle.....degrees | 93               | 110            |
| Tensile Strength.....             | 63.8             | 65.0           |
| Elmendorf Tear Strength.....      | 127              | 80             |

It is to be understood that changes and variations may be made without departing from the spirit and scope of the invention as defined in the appended claims.

I claim:

1. As an article of manufacture, a textile material comprising cellulose fibers cross-linked by impregnation

8

with an aqueous acidic solution of a water-soluble salt of an acid with an amine of the formula



5. where

n is an integer having a value of 2 to 3,

R is a member selected from the group consisting of cyclohexyl, benzyl, and alkyl groups having 1 to 8 carbon atoms,

10 A is an alkylene group having 2 to 4 carbon atoms, and

X is a member selected from the group consisting of O and S,

15 and subsequent heating of the impregnated material at a temperature of about 250° to 400° F. until cross-linking of the cellulose is obtained.

2. An article of manufacture as defined in claim 1 in which the textile material comprises cotton fibers cross-linked as defined in claim 1.

20 3. An article of manufacture as defined in claim 1 in which the textile material comprises regenerated cellulose fibers cross-linked as defined in claim 1.

25 4. As an article of manufacture, a textile material comprising cellulose fibers cross-linked by impregnation with an aqueous acidic solution of a water-soluble salt of an acid with methyl(di-(2-vinyloxyethyl))amine and subsequent heating of the impregnated material at a temperature of about 250° to 400° F. until cross-linking of the cellulose is obtained.

30 5. As an article of manufacture, a textile material comprising cotton fibers cross-linked by impregnation with an aqueous acidic solution of a water-soluble salt of an acid with methyl(di-(2-vinyloxyethyl))amine and subsequent heating of the impregnated material at a temperature of about 250° to 400° F. until cross-linking of the cellulose is obtained.

35 6. As an article of manufacture, a textile material comprising regenerated cellulose fibers cross-linked by impregnation with an aqueous acidic solution of a water-soluble salt of an acid with methyl(di-(2-vinyloxyethyl))amine and subsequent heating of the impregnated material at a temperature of about 250° to 400° F. until cross-linking of the cellulose is obtained.

40 7. As an article of manufacture, a textile material comprising cellulose fibers cross-linked by impregnation with an aqueous acidic solution of a water-soluble salt of an acid with tri(2-vinyloxyethyl)amine and subsequent heating of the impregnated material at a temperature of about 250° to 400° F. until cross-linking of the cellulose is obtained.

45 8. A process of treating a fabric of cellulose fibers which comprises impregnating the fabric with an aqueous acidic solution of a water-soluble salt of an acid with an amine of Formula I and subsequently heating the impregnated fabric at a temperature of about 250° to 400° F. until cross-linking of the cellulose is obtained, Formula I being



60

where

n is an integer having a value of 2 to 3,

R is a member selected from the group consisting of cyclohexyl, benzyl, and alkyl groups having 1 to 8 carbon atoms,

65 A is an alkylene group having 2 to 4 carbon atoms, and X is a member selected from the group consisting of O and S.

70 9. A process as defined in claim 8 in which the salt is that of formic acid.

10. A process as defined in claim 8 in which the salt is that of sulfuric acid.

75 11. A process as defined in claim 8 in which the salt is that of nitric acid.

12. A process as defined in claim 8 in which the salt is that of perchloric acid.

13. A process as defined in claim 8 in which the salt is that of acetic acid.

14. A process as defined in claim 8 in which the salt is that of a mixture of formic and sulfuric acids.

15. A process of treating a fabric of cellulose fibers which comprises impregnating a fabric of cellulose fibers with an aqueous acidic solution containing about 5 to 20% of a water-soluble salt of an acid with an amine of Formula I and subsequently heating the fabric at a temperature of about 250° to 400° F. until cross-linking of the cellulose is obtained, Formula I being



where

*n* is an integer having a value of 2 to 3,

*R* is a member selected from the group consisting of cyclohexyl, benzyl, and alkyl groups having 1 to 8 carbon atoms,

*A* is an alkylene group having 2 to 4 carbon atoms, and *X* is a member selected from the group consisting of O and S.

16. A process as defined in claim 15 in which the fabric is a cotton fabric.

17. A process as defined in claim 15 in which the fabric is a regenerated cellulose fabric.

18. A process of treating a fabric of cellulose fibers which comprises treating a fabric of cellulose fibers with an aqueous acidic solution containing about 5 to 20% of a water-soluble salt of an acid with methyl(di-(2-vinyloxyethyl))amine and subsequently heating the fabric at a temperature of about 250° to 400° F. until cross-linking of the cellulose is obtained.

19. A process of treating a fabric of cellulose fibers which comprises treating a fabric of cellulose fibers with an aqueous acidic solution containing about 5 to 20% of a water-soluble salt of an acid with tri(2-vinyloxyethyl)amine and subsequently heating the fabric at a temperature of about 250° to 400° F. until cross-linking of the cellulose is obtained.

References Cited in the file of this patent

UNITED STATES PATENTS

|           |          |       |               |
|-----------|----------|-------|---------------|
| 2,727,020 | Melamed  | ----- | Dec. 13, 1955 |
| 2,734,890 | Bortnick | ----- | Feb. 14, 1956 |
| 2,734,891 | Melamed  | ----- | Feb. 14, 1956 |